

## UNITED STATES PATENT OFFICE

1,956,899

## ADHESIVE

Jacques Goldmann, Strasbourg, France, assignor  
to Armand Levy, Strasbourg, France

No Drawing. Application April 13, 1932, Serial  
No. 604,921. In France April 18, 1931

2 Claims. (Cl. 87—17)

My invention relates to a glue which adheres to all kinds of materials, and can readily be removed again from them without leaving spots, said glue being moreover not subject to harden and therefore can be used for indefinite time.

The glue of this character especially suits for securing letters, ciphers or other signs to backings, a pad of glue being, to this effect, placed on the object to be secured and the latter pressed on the backing. If they are to be removed again, a short and energetical pulling on the objects will be sufficient. I have found out, that by using characters of concave-convex shape pressed out of thin sheet metal, I obtain the best results, since in such characters the adhering surface of the glue is of larger size than that of the flat backing to which they are secured and therefore the glue pad always remains sticking to the character, when the latter is removed from the backing.

My invention also relates to the manufacturing of the glue.

According to the invention, the glue comprises a composition of:

3.265 kilos of white crepe rubber  
3.605 kilos of factis  
0.400 kilos of resin  
1.300 kilos of benzene  
5.167 kilos of methylhexalinhydrogenester of  
adipic acid  
10.815 kilos of chalk

the rubber and factis being mixed up at a temperature of 75—80° C., the benzene and resin also being mixed up separately and then added to the rubber mixture. Finally the methylhexalinhydrogenester of adipic acid is added for the same purpose as the resin mixture i. e. for liquefying the mass and then the chalk in order to obtain a pasty consistency.

I claim:

1. A glue adhering to all kind of materials comprising a composition of:

3.265 kilos of white crepe rubber

3.605 kilos of factis

0.400 kilos of resin

1.300 kilos of benzene

5.167 kilos of methylhexalinhydrogenester of  
the adipic acid

10.815 kilos of chalk.

2. A process of manufacturing the glue according to claim 1, consisting in mixing up at a temperature of 75—80° C. the rubber and the factis, in mixing up the benzene and resin, in adding the latter to the former mixture, in liquefying the whole mixture by addition of the methylhexalinhydrogenester of the adipic acid and in then adding the chalk.

JACQUES GOLDMANN.

85

90

95

100

105

110

35

40

45

50

55